

# UNITED STATES PATENT OFFICE.

EMILE GEORGES LEGRAND, OF STE. ADRESSE, FRANCE.

## PROCESS FOR PRECIPITATING COPPER-AMMONIA SOLUTIONS OF CELLULOSE FOR THE PURPOSE OF MANUFACTURING ARTIFICIAL-SILK THREADS OR SIMILAR PRODUCTS.

1,130,830.

Specification of Letters Patent.

Patented Mar. 9, 1915.

No Drawing.

Application filed August 29, 1912. Serial No. 717,677.

To all whom it may concern:

Be it known that I, EMILE GEORGES LEGRAND, a citizen of the Republic of France, and resident of Ste. Adresse, France, have invented new and useful Improvements in Processes for Precipitating Copper-Ammonia Solutions of Cellulose for the Purpose of Manufacturing Artificial-Silk Threads or Similar Products, which improvements are fully set forth in the following specification.

The use of caustic alkalis as coagulating agents for cupro-ammonium solutions of cellulose is well known.

15 In prior processes it has been customary to subject solutions of cellulose to the action of concentrated soda lyes, thereby precipitating threads of cupro-cellulose, which latter are caused to pass under pressure 20 through suitable capillary orifices. The products obtained after neutralizing and washing, are supple and transparent. Their strength and elasticity are greater than those of products prepared by precipitation 25 with acids. Nevertheless, this process has in practice important disadvantages. During the spinning, the bath gradually acquires a blue color owing to the presence of copper salts in solution. After a little time, it becomes 30 so colored that it is difficult to see and to tie together the broken threads. At the first washing, the upper layers of thread, in direct contact with water, gradually become whiter and the bottom layers 35 remain dark blue. This results in great irregularity in the quality of the fibers. The whitish portions produce a dull and opaque thread, certain strands remaining shiny and crystalline, while others have an opalescent 40 milky appearance. These irregularities reappear in the dyeing; the thread is spotted, and on testing there are also found differences in the strength and elasticity.

This invention relates to the addition, to 45 the alkalis, of diastase solutions capable of decoloring the caustic soda solution by reducing copper salts in solution, and of reinforcing or strengthening the cellulose fiber by completing the coagulation obtained by 50 means of the alkaline lyes. Such a solution added in proportions of 4% to the spinning bath, produces very important new technical effects.

1. In the presence of hot concentrated 55 caustic soda solution preferably between 40

and 45° C. (the reaction is still possible from 45-50° C.), the diastase acts as an energetic reducing agent. This temperature of the bath is indispensable, for, unlike other reducing agents with aldehydic or ketonic functions (glycerin, poly-saccharid sugar, etc.) which act only at the temperatures of 45-75° C., the diastase in alkaline medium does not act above 70° C. From 50-70° C. its reducing and coagulating 60 property gradually decreases. At 75° C. the diastase is completely decomposed. It is therefore necessary that the temperature of coagulation should not exceed 50° C. Beginning with 40° C., the copper salts in 70 solution are precipitated, the caustic soda solution assumes gradually a reddish color, enabling the blue threads to be easily guided and tied together in the precipitating bath. The copper oxid settles at the bottom of the 75 vats; it is withdrawn by decanting and recovered in the state of precipitated copper.

2. The spools charged with cupro-cellulose precipitated by the mixture of caustic soda and diastase in solution, have 80 uniformly the same appearance. The thread, on coming out from spinning, has a dark green color which it retains even after a long washing with water. As soon as it has been deprived of copper, it keeps 85 all its transparency and has a bright color. The strands do not contain either dull or spotted portions, the dyeing is very regular and especially brilliant.

3. By the addition of diastase to caustic 90 lyes, the coagulating action of the precipitating bath is strengthened and lengthened, the resistance and, more particularly, the elasticity of the thread are increased. Dynamometric tests clearly show the reinforcing action of diastase on the silk in alkaline medium. With a spinning bath of concentrated caustic soda of 40% with 4% of diastase, the silk thus coagulated gives a mean elasticity of 22%. With the caustic soda 100 solution alone, of the same degree of concentration, the average elasticity is only 14%. Owing to this flexibility, the artificial silk approaches very nearly to natural silk. Its strength and elasticity considerably increased by this process, enable it to find a ready market, more particularly in mechanical embroidery and weaving.

According to the process forming the subject of this invention, the same results can 110

be obtained by the simultaneous use of diastase and of diluted alkaline lyes. It is preferable to use as a precipitating bath weak caustic soda containing 16-21% NaOH

5 with the addition of 3, 4 or 5% diastase.

Up to now, in all processes relating to the precipitation of cupro-ammonium solutions of cellulose by caustic alkalis, it is specified that the coagulating liquids are concentrated 10 caustic soda solution or potash lyes, whether the caustic soda in question be used alone or mixed with caustic soda salts or contain an addition of poly-saccharids and aldehyde alcohols, formaldehyde, glycerin, glucose, 15 saccharose, lactose, sucrate of lime, etc.

Claims:

1. The improvement in processes of the kind described which consists in subjecting

cupro-ammonium solutions of cellulose in suitable form to a bath comprising a solution of caustic alkaline lye and diastase for the purpose described. 20

2. The improvement in processes of the kind described which consists in subjecting cupro-ammonium solutions of cellulose in suitable form to a bath composed of a weak solution of caustic lye and diastase for the purpose described. 25

In testimony whereof I have signed this specification in the presence of two sub- 30 scribing witnesses.

EMILE GEORGES LEGRAND. [L. S.]

Witnesses:

G. HOADLEY,  
CONSTANT GUÉRARD.